

Sept. 15, 1942.

R. T. FIELDS

2,295,942

MANUFACTURE OF FILAMENTS

Filed Aug. 2, 1940



Reuben T. Fields

INVENTOR

BY *J. W. Castle Jr.*

ATTORNEY

## UNITED STATES PATENT OFFICE

2,295,942

## MANUFACTURE OF FILAMENTS

Reuben T. Fields, Arlington, N. J., assignor to E. I.  
du Pont de Nemours & Company, Wilmington,  
Del., a corporation of Delaware

Application August 2, 1940, Serial No. 349,840

5 Claims. (Cl. 18—8)

This invention relates to the manufacture of filaments and, more particularly, to the manufacture of relatively coarse filaments of synthetic linear condensation polymers by melting and spinning the polymers.

By the term "synthetic linear condensation polymers" is meant new polymeric materials such as described in United States Patents 2,071,250 and 2,071,253, and in United States application Serial No. 136,031, filed April 9, 1937, now Patent No. 2,130,948, all of W. H. Carothers.

These synthetic linear condensation polymers are subject to destructive change at the elevated temperatures at which they become molten. A tendency to undesired further polymerization during the steps of melting and spinning is minimized by limiting the dimensions of the equipment used in these steps and thereby limiting the duration of exposure of the material to high temperature. A further result of exposure to high temperature is a slow chemical decomposition, which results in the release of gaseous products.

It has been recognized, in connection with any and all spinning of filaments of these materials, that the presence of bubbles of gas, coming from decomposition, or from simple entrapment from the atmosphere of the vessel in which the polymer is melted, is definitely objectionable since, if such bubbles are carried through to the spinneret, they are likely to result in broken or defective filaments, or otherwise cause irregularities in the operation of spinning. In a copending application of Graves, Serial No. 232,314, filed September 29, 1938, now Patent No. 2,278,875, provision has been made, by compressing the molten synthetic linear polymer, to redissolve any gaseous decomposition products and to prevent the further formation of bubbles in the molten mass, and to deliver the molten mass, free from bubbles, by a suitable metering device to the spinneret.

Thus to dissolve gases in the molten polymer by application of high pressure is practicable and satisfactory in result in connection with the spinning of filaments of the very small diameters required for ordinary textile purposes, both because high pressures must ordinarily be imposed upon the molten polymer to overcome the frictional resistance of the spinneret and its ac-

cessories to the spinning of fine filament at commercial rates, and also because the smallness of the diameter of such filament permits it to be so rapidly hardened by chilling, as it emerges from the spinneret, that gases dissolved in it are not released, and no bubbles are formed.

In the manufacture of coarse filaments, such as those used as monofilaments for bristles, sutures, fish-line leaders, racquet strings, et cetera, the specific problem is rather different. Filaments of the much larger diameters here involved, of the order of 0.020 inch (undrawn) and upward, and particularly of 0.040 (undrawn) inch and upward, are so much less rapidly chilled through, after emerging from the spinneret, that gases previously dissolved in the molten mass by application of high pressure have opportunity to become released during the time between the release of the pressure at the exit of the spinneret and the effective solidification of the filament.

Particularly troublesome is water dissolved in the melt as a result of its presence in the initial polymer and of a failure to expel it from the molten mass.

Broadly, it is the object of the present invention to provide equipment and procedure whereby to spin, from synthetic linear condensation polymers, coarse filaments of uniform diameter and free from bubbles and discoloration.

More specific objects are to provide equipment and procedure to effect melting of the polymers without access of oxygen, to minimize the duration of exposure of the molten material to temperatures capable of causing its decomposition, to deliver molten material bubble-free to the spinneret under uniform pressure, and to conduct the process as a whole, from melting to spinning, under minimum pressure, in order to minimize the content of releasable gases within the molten material.

A further object of the invention is to provide equipment which is adapted to handle molten polymer over a wide range of consistency and over a wide range of initial admixture with gas, and to provide so effectively for the escape of water vapor that it is adapted to handle initially wet polymer. Other objects will be apparent from the description of the invention given hereinafter.

The above objects are accomplished according to the present invention by a process which comprises melting a synthetic linear condensation polymer while blanketed with carbon dioxide to the exclusion of oxygen and at no greater than atmospheric pressure, introducing the melted polymer into a screw pump having a capacity at its intake end several times greater than its capacity at its discharge end, and delivering said molten polymer under pressure to a spinneret to cause the molten polymer to pass through the orifice of the spinneret and emerge as a filament, the polymer being kept out of contact with oxygen from the time it is melted until its emergence from the spinneret as a filament.

The melted polymer may be forced through the spinneret either by the pressure developed in the screw pump or by auxiliary pumping means interposed between the screw pump and the spinneret. The filament should be rapidly cooled as it is extruded and this is preferably accomplished by bringing it into contact with water.

By "capacity" of the screw pump is meant the volume of material forwarded per turn of the screw, assuming geometrically perfect delivery with no compression or slippage. To carry out the present invention the capacity of the screw pump must be several times as great at its intake end as at its delivery end, preferably in a ratio of not less than 4 to 1. Although the screw pump may be constructed so that its change in capacity from end to end is gradual, it is usually more convenient to construct the screw pump so that the capacity is changed abruptly at some point along the screw and this type of screw pump is preferred.

In the preferred form of apparatus according to the present invention, the screw pump is used to deliver the molten polymer directly to the spinneret without any interposed auxiliary pumping means. In such apparatus, not only is the ratio of the capacity of the screw pump at its intake end and delivery end important but, also, it is important that the depth of the flute of the screw, at the delivery end particularly, should not exceed .150" in any screw pump of suitable size and proportions for use for this purpose. This will be more fully discussed hereinafter. By "depth of the flute" is meant the distance, measured radially, from the floor of the flute in the screw to the inner surface of the casing of the screw pump. Practically, the depth of this flute should be between .050" and .150". If an unusually viscous melt were to be pumped, the depth of the flute might be slightly greater.

The present invention resides in the discovery that proceeding as described above coarse filaments of .010" diameter and greater, especially those filaments of .020" diameter and greater, undrawn, may be readily extruded without flaws whereas applicant has been unable to find any other practical way of manufacturing such coarse filaments without encountering flaws therein, presumably caused by the release of gas dissolved in the polymer prior to its extrusion. The procedure of the present invention is carefully designed to reduce the gases absorbed by the molten polymer to such a minimum that they are not released from the extruded filament.

In the drawing forming a part of the present application, the figure of the drawing is a vertical section, more or less diagrammatical, of an apparatus constructed according to the preferred form of this invention.

Referring to the drawing, the synthetic linear

condensation polymer is melted in a heated chamber 11 which is desirably of cylindrical shape with a truncated conical bottom and is provided with a cover 12 containing a port 13 through which the polymer may be fed into the chamber. In the lower part of the chamber 11 are banks of tubes 14, 14 running at right angles to each other and adapted to carry a heating fluid for melting the polymer. The cylindrical sides and conical lower portion of the chamber are enclosed in a jacket 15 similarly adapted to carry a heating fluid in circulation, and the tubes 14, 14 preferably communicate with this jacket so that a single source of heating fluid will provide the circulation thereof in both jacket and tubes.

The heating chamber 11 is provided also with means for the entry and escape of the blanketing gas. Conveniently, these take the form of pipes passing through the cover 12 and, preferably, the intake pipe 16 extends downward within the chamber nearly to the level of the uppermost of the banks of tubes while the outlet pipe 17 is located near or in communication with the port 13. Throughout the operation of the equipment, the blanketing gas, carbon dioxide, is fed into the chamber 11 through the pipe 16 and flows out of the chamber either through the pipe 17 or, if the port 13 is open, then also through this port. By this means, air is excluded from the interior of the chamber 11 while it is in operation and the polymer is protected against contact with air throughout the duration of its stay in this chamber without using superatmospheric pressure. Water vapor also escapes with the carbon dioxide.

While the constant escape of blanketing gas can be relied upon to prevent the entry of air into the chamber 11 through the port 13 when the latter is open, it is desirable that the feeding port 13 be provided with a cover 18 and that this be kept in place whenever the port is not being used for feeding. When this cover 18 is in place, the blanketing gas escapes through the outlet pipe 17. The blanketing gas is fed into the chamber 11 merely at a rate which is fast enough to insure against the entry of air through the port 13, the discharge pipe 17, or any other possible point of entry.

An opening at the bottom of the truncated conical portion of the chamber 11 communicates with an opening into the casing 19 of a screw pump of special design. This casing 19 is provided with a jacket 20 for the circulation of a heating fluid, this jacket 20 and the jacket 15 of the heating chamber intercommunicating through a duct 21. This closed circulating system is provided with an inlet 22 in the jacket 15 and with an outlet 23 in the jacket 20 for return of the heating fluid to the source of heat.

The interior wall of the casing 19 of the screw pump is accurately cylindrical. Within it, with clearance as hereinafter described, rotates the screw member 24 which, at the intake end of the screw pump, is extended through the casing 19 to constitute a shaft 25 by which the screw member 24 may be rotated through a chain drive actuating a pulley or sprocket 26 keyed to this shaft 25.

Within the casing 19, at the intake end, the screw member 24 carries a double-lead flute 27 which terminates in a circumferential groove 28. From this point on, to the discharge end of the screw pump at 29, the screw member 24 carries a single-lead flute having a capacity substantially less than that of the double-lead flute 27.

The dimensions of the screw pump may suitably be as follows:

|                                           | Inches |
|-------------------------------------------|--------|
| Total length of screw                     | 15     |
| Length of screw with double-lead flute    | 4      |
| Length of screw with single-lead flute    | 11     |
| Depth of double-lead flute                | 0.125  |
| Width of double-lead flute                | 0.250  |
| Pitch of double-lead flute                | 0.667  |
| Depth of single-lead flute                | 0.063  |
| Width of single-lead flute                | 0.250  |
| Pitch of single-lead flute                | 0.333  |
| Inside diameter of casing                 | 1.625  |
| Clearance between screw and casing, about | 0.0025 |

Rotation of the screw member 24 serves to convey molten polymer, falling from the surfaces of the tubes 14, 14 into the casing of the screw pump, from the intake end of the latter to the discharge end at 29. The manner of operation of this screw member 24 will be more completely described hereinafter.

The discharge end of the pump at 29 communicates, through suitable channels, with a spinneret 30 through which, by the pressure generated, as hereinafter described, by the screw member 24 within the casing 19, the molten polymer is extruded to form filaments and the like.

As shown in the drawing, the channel communicating with the spinneret 30 is contained within a block 31 attached to the casing 19 of the screw pump at the discharge end. A hole drilled through this block, parallel with the axis of the screw member 24, forms a channel 32 which at its entrance end is in communication with the interior of the screw pump and which at its opposite end is in communication, through a diaphragm, with a pressure gauge 33.

A second hole cut in the block 31, conveniently at right angles with the channel 32 and not extending through the block, constitutes a channel 34 which serves to connect the channel 32 with the spinneret 30.

Molten polymer enters the casing 19 of the screw pump from the heating chamber 11 and is carried along in the direction of the spinneret by the rotation of the screw member 24. It is preferred to rotate the screw member 24 at about 350 R. P. M. although it may be rotated anywhere between 100 R. P. M. and 400 R. P. M. The decrease in the flute capacity of the screw member 24 exerts a compressive action upon the molten polymer and thereby causes the disappearance of bubbles which have become entrapped in the course of the melting of the polymer upon the tubes 14, 14. The gas becomes completely dissolved in the molten polymer.

It is because of the voluminousness of the molten mass entering the pump that the diminishment in the capacity of the pump from intake to discharge end should preferably be made in a ratio of at least 4 to 1.

When the entire system, comprising the screw pump, the channels 32 and 34, and the spinneret fixture 30, has become filled with molten polymer, the propulsive and compressive action of the screw pump builds up a pressure upon the molten material in the channels and spinneret, and this pressure effects the extrusion of molten material through the orifice or orifices of the spinneret. The magnitude of this pressure influences the rate at which the molten material is extruded and constitutes a minor influence upon

the diameter of the filaments produced by a spinneret of given diameter of orifice. The important influences on the diameter are the linear rate at which the filament produced is carried away from the spinneret and the rate of rotation of the pump screw.

It will be understood that the design of the screw pump as illustrated in the drawing and the dimensions thereof given above are merely illustrative and that both the design and dimensions may be varied considerably without departing from the scope of this invention.

Nevertheless, since the pump must serve to compress the molten polymer and redissolve any entrapped gas as well as furnish the pressure for extruding the polymer, which pressure, however, need not exceed 75 pounds per square inch, it must possess certain characteristics to function satisfactorily.

The action of the screw pump on the molten polymer, which is a viscous liquid, may be likened to rolling a pencil between the palms of the hands with one palm held stationary. That is, the molten polymer is, in effect, rolled between the stationary inner surface of the pump casing and the moving floor of the flute in the screw. From this analogy, it will be apparent why the depth of the flute is such an important factor in the design of the pump. The depth of the flute should be between .050" and .150".

The side walls of the flute offer resistance to the desired motion of the molten polymer and, for this reason, the flute must not be too narrow; it has been found that the width of the flute should not be less than about 0.125 inch, and preferably not less than about 0.25 inch.

On the other hand, the width of the flute should not be too great, since on a screw of reasonable length the path of the flute would be shortened thereby too much to prevent back flow of the molten polymer. For this reason, the width of the flute on a screw of the length and diameter described above, i. e., 15 inches and 1.625 inches, respectively, should not exceed about 0.50 inch.

This is approximately one third of the diameter of the screw, and it has been found to be a desirable rule that the width of the flute shall not exceed one third of the diameter, regardless of what the diameter may be. At a fixed ratio of width of flute to diameter of screw, a change in the latter does not appreciably change the length of path of the flute upon a screw member of given length, nor does it change the angle of the flute with respect to a longitudinal element of the screw member. The limiting ratio of one to three provides for an adequately long path upon a screw member of reasonable length, and also avoids the loss of efficiency which results when this angle is too small.

The diameter of the screw member will, for practical reasons, be ordinarily between about one inch and three inches. For reasons of rigidity and torsional strength it must not be too small, whereas on the other hand there is no point in making it too large, since the corresponding increase in peripheral speed, at a given rotational speed, tends to increase the intensity of friction upon and within the molten polymer and thus to cause objectionable overheating.

A combination of the narrowest feasible flute (stated above to be about 0.125 inch) upon a screw member of the smallest feasible diameter (stated above to be one inch), represents a ratio, of width of flute to diameter of screw, of one

to eight. But in general, particularly on screws of larger diameters, the ratio may permissibly be as low as one to ten.

Thus the width of the flute is conveniently expressed in terms of the diameter of the screw member, as being between one tenth and one third of that diameter. In the case of a screw member of diameter 1.625 inches, such as that described above, the preferred range of width of flute, i. e., 0.25 to 0.50 inch, lies within this somewhat broader range.

The pitch of the screw, ordinarily, will be automatically determined by the width of the flute employed because the width of the "land" between successive convolutions of the flute will be made as narrow as efficiency in sealing between convolutions of the flute and acceptable resistance to wear will permit; increasing the width of the "land" beyond this point would be simply uneconomical as it would serve no good purpose. It has been found that a width of .050 for the "land" is sufficient both to give adequate resistance to wear and to seal the flute effectively.

If auxiliary pumping means such as a gear pump is to be interposed between the screw pump and the spinneret, a feasible but not preferred embodiment of the invention, for the purpose of furnishing the desired pressure for extruding the molten polymer through the spinneret, more leeway is permitted in the design of the screw pump because the screw pump is then only required to compress the molten polymer and dissolve the entrapped gases, not to deliver the polymer at a pressure high enough to extrude it through the spinneret. Also, at the intake end of the screw pump, the dimensions of the flute in the screw need not be within the limits discussed above although it is preferred that they should be.

With respect to other parts of the apparatus shown in Fig. 1, various modifications without departing from the scope of the invention will be apparent to those skilled in the art. The heating chamber 11 may be widely varied in design providing only that it is adapted to effect the melting of the polymer at atmospheric pressure while the polymer is completely blanketed with carbon dioxide gas. Connecting the heating jackets 15 and 20 is obviously a matter of convenience since independent heating jackets would function just as well.

The specific construction of the spinneret 30 forms no part of the present invention. The construction of these spinnerets is well known in the art and the selection of a suitable one will be based on considerations not involving the present invention.

The present invention has been described in connection with the melting and spinning of synthetic linear condensation polymers of which polyhexamethylene adipamide is a prominent specific member. Actually, the invention is applicable to the melt-spinning of any organic filament-forming composition which is subject to the formation of bubbles under the conditions existing during its melting and spinning. The synthetic linear condensation polymers include synthetic linear polyamides, that is, synthetic linear polymers containing  $-\text{CONH}-$  units in the linear chain, synthetic linear polymers such as polyesters, polyethers, polyacetals, and mixed polyester-polyamides, such as may be prepared by condensation reactions as described in United States Patent 2,071,250.

The filament-forming material used in accord-

ance with the present invention may contain modifying agents, e. g., luster-modifying agents, plasticizers, pigments, dyes, antioxidants, resins, et cetera. The present invention may be used to advantage in the handling of compositions in which the formation of bubbles may be caused by the presence of a modifying agent.

The invention provides a method and an apparatus whereby organic filament-forming compounds, and compositions comprising them, can be spun into coarse filaments of uniform diameter, free from bubbles and discoloration. The apparatus is simple, and the relatively low pressures involved make for economy of construction and safety in operation. Furthermore, the invention makes feasible the use of polymer of high content of moisture.

As many apparently widely different embodiments of this invention may be made without departing from the spirit and scope thereof, it is to be understood that the invention is not limited to the specific embodiments thereof except as defined in the appended claims.

I claim:

1. Process of preparing coarse filaments of at least .020" diameter from a synthetic linear condensation polymer, which comprises melting said polymer while blanketed with carbon dioxide gas under a pressure not exceeding atmospheric pressure, introducing the molten polymer into a screw pump having a capacity at its intake end several times greater than its capacity at its discharge end, and delivering said molten polymer under pressure to a spinneret to cause said molten polymer to be extruded therethrough in the form of a filament.

2. Process of preparing coarse filaments of at least .020" diameter from a synthetic linear condensation polymer, which comprises melting said polymer while blanketed with carbon dioxide gas under a pressure not exceeding atmospheric pressure, introducing the molten polymer into a screw pump having a capacity at its intake end at least four times as great as its capacity at its discharge end, and delivering said molten polymer under a pressure of about 75 pounds per square inch to a spinneret to cause said molten polymer to be extruded therethrough in the form of a filament.

3. Apparatus for preparing coarse filaments from a synthetic linear condensation polymer, which comprises a chamber for melting said polymer, means for heating said chamber, means for introducing an inert gas heavier than air into said chamber to blanket at least the lower portion thereof, a screw pump disposed below said chamber and having its intake end communicating with the bottom of said chamber, and a spinneret in communication with the discharge end of said screw pump, said screw pump having a capacity at its intake end at least four times as great as its capacity at its discharge end and comprising a screw provided at the discharge end with a flute between .050" and .150" in depth and .25" and .50" in width.

4. Apparatus for preparing coarse filaments from a synthetic linear condensation polymer, which comprises a chamber open to the atmosphere for melting said polymer, means for heating said chamber, means for introducing an inert gas heavier than air into said chamber to blanket at least the lower portion thereof, a screw pump disposed below said chamber and having its intake end communicating with the bottom of said chamber, and a spinneret in communication with the discharge end of said screw pump, said screw

pump having a capacity at its intake end at least four times as great as its capacity at its discharge end and comprising a screw between 1.0" and 2.0" in diameter and provided at the discharge end with a flute between .050" and .150" in depth and .25" and .50" in width.

5. Apparatus for preparing coarse filaments from a synthetic linear condensation polymer, which comprises a chamber open to the atmosphere for melting said polymer, means for heating said chamber, means for introducing an inert gas heavier than air into said chamber to blanket at least the lower portion thereof, a screw pump

disposed below said chamber and having its intake end communicating with the bottom of said chamber, and a spinneret in communication with the discharge end of said screw pump, said screw pump having a capacity at its intake end at least four times as great as its capacity at its discharge end and comprising a screw between 1.0" and 2.0" in diameter and provided at the discharge end with a flute between .050" and .150" in depth and between one-tenth and one-third of the diameter of the screw in width.

REUBEN T. FIELDS.